

## UNITED STATES PATENT OFFICE

2,443,823

## SULFURIZED TERPENES

Lee Cone Holt, Wilmington, Del., assignor to E. I. du Pont de Nemours & Company, Wilmington, Del., a corporation of Delaware

No Drawing. Application March 2, 1945,  
Serial No. 580,709

12 Claims. (Cl. 260—139)

1

This invention relates to non-corrosive sulfurized terpene products, processes for preparing the same and lubricants containing them.

The reaction of sulfur with terpene hydrocarbons to form sulfurized products has been known for many years. Such sulfurized products contain terpene sulfides and considerable amounts of highly reactive or corrosive sulfur generally present either as dissolved sulfur or as polysulfides or both. The terpene sulfides produced are of unknown structure and are usually admixed with by-product hydrocarbons including *p*-cymene. Such sulfurized products have been concentrated by distillation to yield residues containing large amounts of sulfur, which is very corrosive, but which does not crystallize from the products. P. O. Powers, in Patent 1,926,648, has proposed to wash a sulfurized terpene hydrocarbon product free of corrosive and odiferous impurities with aqueous sodium hydroxide solution.

The sulfurized terpene products, obtained by the methods of the prior art, are known to be useful in cutting oils. However, prior to my invention, no one has produced a sulfurized terpene product which has been satisfactory for commercial utilization in automotive lubricants and the like. One of the main reasons for this has been that such products are too corrosive for such use. The best of such products tend to cause pitting of alloy bearings with resultant bearing losses when employed in an engine. Such pitting is objectionable. Most of such prior products, and particularly those prepared from pinene and pine oil, are characterized by bad color, the presence of substantial amounts of insoluble materials and are somewhat unstable at elevated temperatures.

It is an object of my invention to provide non-corrosive sulfurized terpene hydrocarbon products useful as additives for automotive and like petroleum lubricating oils and which will impart beneficial properties to such oils. Another object is to provide a novel method for producing non-corrosive sulfurized terpene hydrocarbon products. A further object is to provide new and improved lubricants. Other objects are to provide new compositions of matter and to advance the art. Still other objects will appear hereinafter.

The above and other objects may be accomplished in accordance with my invention which comprises, in part, the steps of sulfurizing at least one terpene of the class of dipentene and terpinolene and washing the reaction product at about 85° C. to about 100° C. with an aqueous solution of an alkali metal sulfide of about 20% to about 30% concentration until a sulfurized terpene product is obtained, which, in 1% concentration in petroleum oil, will be substantially non-staining to

metallic copper when maintained in contact therewith for 3 hours at 100° C. The resulting products are new and valuable, particularly for use in petroleum oils employed for automotive and like lubrication. Preferred products, however, are obtained by topping the washed product, under vacuum to a pot temperature within the range of from a minimum temperature of about 100° C. to a maximum temperature of about 5° C. above the sulfurizing temperature, until the concentration of sulfur in the product is increased to from about 24% to about 36%. These preferred products are particularly valuable for use in petroleum oils employed for automotive lubrication.

As a means of measuring the reactivity of the sulfur in products of this character and their suitability for use in automotive lubricants and the like, I have employed the copper strip test. In this test, the sulfurized product is dissolved in a petroleum lubricating oil to provide a solution containing an amount of sulfur ordinarily desired for lubricants of this character. A polished copper strip is exposed to such solution for 3 hours at a given temperature. Thereafter, the color of the copper strip is compared with the color of a standard set of copper strips. The standard strips are numbered from 1 to 10, varying in color from the original copper to black, as follows:

1. Original copper
2. Slight yellow stain
3. Light bronze<sup>1</sup>
4. Medium bronze<sup>1</sup>
5. Dark bronze<sup>1</sup>
6. Weathered copper—purplish
7. Dark weathered copper—red brown—no black
8. Dark weathered copper, with light layer of black soot
9. Dark weathered copper with black areas
10. Black film

Since the staining of the copper strip is due to the formation of copper sulfide, this is a very delicate test for sulfur reactivity. The tendency of an additive to corrode copper parts in normal engine operating conditions is indicated by testing in the above test at 210° F. All tests given hereinafter are at 210° F. for 3 hours, except where otherwise indicated. To obtain comparable sulfur concentrations, I have generally tested the washed, not topped, oils at 1% concentrations on the lubricant and the topped additives at ½% concentration on the lubricant. In general, blends of product, giving copper strip values of 5 or less, may be used in lubricants without excessive corrosion under normal operating conditions, although for some types of service, lower values are desirable. This copper strip test is

60 <sup>1</sup>Bronze refers to natural color of polished bronze.

a modification of method 530.31. Corrosion test at 212° F. (copper strip) listed in the Federal Standard Stock Catalog, section 4, part 5. Federal specification for lubricants and liquid fuels; general specifications (methods for sampling and testing), VV-L-791b. Some measure of the availability of the combined sulfur for reaction under excessive load conditions, when higher temperatures are developed, may be obtained by operating the above test at higher temperatures such as 300° F. or other selected temperature.

The terpene hydrocarbons, which are employed to produce the products of my invention, are dipentene, terpinolene and commercial mixtures thereof. While the products may be made from pure dipentene and pure terpinolene, I preferably prepare the products from commercial mixtures of terpenes, the major proportion of which consists of dipentene and terpinolene. These commercial mixtures will generally contain from about 65% to about 30% of dipentene and about 5% to about 60% of terpinolene, the rest usually being inert p-cymene and p-menthane. A particularly desirable mixture is that obtained as a by-product in the manufacture of camphor and boiling in the range of about 178° C. to about 195° C. This last mixture appears to be essentially a mixture of about 30% dipentene, about 30% terpinolene, about 30% of an isomeric terpene hydrocarbon boiling at about 187° C. to about 188° C., together with minor amounts of menthenes and p-cymene. The isomeric terpene hydrocarbon boiling at 187 to 188° C. is isomeric to the dipentene and the terpinolene and is a full equivalent thereof. I have found that it is possible to obtain products of satisfactory color, stability and solubility from these terpenes and which products are distinctly superior to products obtainable from pinene and pine oil.

The sulfurization will be carried out in the manner usually employed for sulfurizing materials of this character by heating the terpene and sulfur in a temperature range of from about 135° C. to about 180° C. Usually, there will be employed from about 1.5 to about 2.1 atoms of sulfur for each mole of the unsaturated terpene to be sulfurized. Excess proportions of sulfur can be employed but without advantage. Smaller proportions of sulfur can be employed, but with a decrease in yield. In treating mixtures containing inert materials, the proportion of sulfur will be calculated on the basis of the unsaturation of the mixture. The reaction mixture will be maintained at the reaction temperature for a period of from 1 to about 6 hours in order to decompose products which are thermally unstable at the selected reaction temperature.

The crude sulfurized products will contain corrosive sulfur and polysulfide materials which will blacken a copper strip at 100° C. or below and which are highly objectionable. I have found that such objectionable materials can be removed from the crude reaction mixture by washing such reaction mixture with an aqueous solution of an alkali metal sulfide at temperatures of from about 85° C. to about 100° C. Preferably, the alkali metal sulfide will be sodium sulfide. Also, preferably, the aqueous solution will contain the alkali metal sulfide in a concentration of from about 20% to about 30%. The reaction product will be given one or more washes with the sodium sulfide solution and until a product is obtained which, when dissolved in a petroleum oil in a concentration of 1%, will be substantially non-staining to metallic copper at 100° C., that is, will have 75

a value of from 1 to 5 in the copper strip test hereinbefore described. Generally, it will be desirable to first wash the crude reaction product one or more times with aqueous caustic soda at about 85° C. to about 100° C. The preliminary washing with caustic soda will not remove the corrosive and undesirable sulfur and sulfur compounds to the same extent as will the sodium sulfide, but will reduce the amount of sodium sulfide required to remove the undesirable materials to the desired extent.

In order to show the advantages of the washing with sodium sulfide over washing with caustic soda, the crude unwashed sulfurized terpenes of Examples III and II, described hereinafter, were given washes with caustic soda and with sodium sulfide. The crude unwashed sulfurized product of Example III was washed with a 30% aqueous sodium hydroxide solution by agitating it with the solution for 1.5 hours at 90° C. This washed product was then divided into 2 portions. One portion was further washed with 5 washes of 30% sodium hydroxide solution at 90° C., employing 1.5 hours agitation in each case. The second portion was washed 5 times in the same manner with an equivalent amount of aqueous 24% sodium sulfide solution. The results are given in Table 1:

TABLE 1

|                              | Per Cent S | Refractive Index 90° C. |
|------------------------------|------------|-------------------------|
| After 1-NaOH Wash            | 18.97      | 1.5380                  |
| Oil Split into Lots 1 and 2: |            |                         |
| Lot 1 after—                 |            |                         |
| 2d NaOH Wash                 | 18.3       | 1.5360                  |
| 3d NaOH Wash                 | 18.4       | 1.5364                  |
| 4th NaOH Wash                | 18.4       | 1.5361                  |
| 5th NaOH Wash                | 18.4       | 1.5351                  |
| 6th NaOH Wash                | 18.3       | 1.5370                  |
| Lot 2 after—                 |            |                         |
| 1st Na <sub>2</sub> S Wash   | 16.6       | 1.5311                  |
| 2d Na <sub>2</sub> S Wash    | 15.6       | 1.5290                  |
| 3d Na <sub>2</sub> S Wash    | 15.5       | 1.5261                  |
| 4th Na <sub>2</sub> S Wash   | 15.1       | 1.5258                  |
| 5th Na <sub>2</sub> S Wash   | 15.2       | 1.5232                  |

The crude unwashed sulfurized product of Example II was washed once with caustic soda, and then divided into two portions. One portion was given 2 additional caustic washes. The other portion was given 2 sodium sulfide washes. The washes were conducted in the same manner as hereinbefore described with respect to the product of Example III. The results of this treatment are shown in Table 2:

TABLE 2

|                                                                             | Per Cent S |
|-----------------------------------------------------------------------------|------------|
| Crude Reaction Oil after 1-NaOH Wash<br>Washed Oil Split into Lots 1 and 2: | 18.5       |
| Lot 1 after—                                                                |            |
| 2nd NaOH Wash                                                               | 17.9       |
| 3rd NaOH Wash                                                               | 18.0       |
| Lot 2 after—                                                                |            |
| 1st Na <sub>2</sub> S Wash                                                  | 17.2       |
| 2nd Na <sub>2</sub> S Wash                                                  | 15.9       |

It will thus be apparent that one washing of the crude reaction product with aqueous alkali metal sulfide reduces the sulfur content of the sulfurized product to a level substantially below that attainable by exhaustive washing with caustic soda alone.

The sulfurized products, as obtained by the washing with sodium sulfide solution, will have a value of 5 or less by the copper strip test hereinbefore described. They are novel materials and are desirable additives for petroleum lubricating

## 5

oils to which they impart desirable characteristics such as extreme-pressure properties and improved oxidation stability at temperatures of from about 110° C. to about 200° C. When prepared from commercial mixtures of terpenes, they contain from about 15% to about 19% sulfur. However, the concentration of sulfur will vary with the proportions of inert materials in the starting mixture and may be somewhat higher or lower. Usually, in products of this character, it is desirable to have higher and more uniform concentrations of sulfur. Also, I have found that the properties of these products can be further improved and that they can be given additional beneficial properties.

The preferred products of my invention will be obtained by subjecting the washed products to distillation under vacuum to remove hydrocarbon materials and terpene mono-sulfides. Such distillation will be sometimes referred to herein and in the claims as "topping." Preferably, the topping will be carried out under vacuum of from about 10 mm. to about 60 mm. Care must be taken in this distillation in order to obtain a product having the desired characteristics for use in automotive lubrication and in order to avoid producing a product which will be too corrosive for such use.

Temperatures of about 100° C. or more will be required to remove the desired amount of hydrocarbon materials. However, if the pot temperature is increased to more than about 5° C. above the highest temperature at which the sulfurization was carried out, there is a tendency toward an undesirable amount of chemical condensation and decomposition to produce products which will contain an objectionable amount of corrosive sulfur so that the product will be too corrosive for use in automotive lubrication. If the pot temperature is maintained at about 125° C. or below during the topping operation, there will be substantially no change in the properties of the product, except those to be expected by concentration of the effective sulfurized material. On the other hand, the topping operation can be carried out at higher pot temperatures to obtain a desired degree of chemical condensation and decomposition of the product with a resultant increase in sulfur activity. This chemical condensation is shown by the formation of terpene mono-sulfide which distills out of the reaction mass. The maximum increase in sulfur reactivity, without obtaining undesirable corrosive materials, will be obtained by topping to a pot temperature within about 5° C. of the reaction temperature employed for sulfurization. Thus, a product, which is formed by sulfurization at 145° C., will show a considerable increase in sulfur reactivity if topped for about 1 hour at temperatures of from about 140° C. to about 150° C., but will show an excessive increase in reactivity if topped to temperatures substantially above 150° C. On the other hand, a product, reacted at 165° C., may be topped to about 145° C. with little increase in sulfur activity, whereas, if it is topped to temperatures of from about 160° C. to about 170° C. for one hour, there will be a desirable moderate increase in sulfur activity and topping to temperatures substantially about 170° C. will give an excessive and undesirable increase in sulfur activity.

Not only is the increase in sulfur reactivity a function of the temperature in the distillation pot in relation to the reaction temperature, but is also a function of the time of heating. There-

## 6

fore, it is essential that the topping operation be extended only sufficiently long to increase the concentration of the sulfur in the product to about 36%. A substantial extension of the topping operation beyond this point, particularly in the higher temperature ranges, tends to result in a product containing an excessive and undesirable amount of corrosive sulfur. Usually, the topping operation, in accordance with my invention, will be carried out until a product is obtained which contains from about 24% to about 36% of sulfur. The copper strip test can also be used to indicate when the product has been excessively cracked during topping. A product, which has been topped to such an extent that it forms a black film on the copper strip, by the copper strip test, is undesirable and has been excessively topped. The topping operation may be aided by passing steam or an inert gas through the product during the distillation.

In order to more clearly illustrate the methods of producing my improved sulfurized terpene products and the products obtained thereby, the following examples are given:

## EXAMPLE I

84 pounds of sulfur were charged to an iron vessel and heated to 150° C. The agitation was started and 241 pounds of terpene hydrocarbons (by-product of boiling range 178-195° C. from the camphor process) were slowly added over a period of 3 hours, the temperature being adjusted to 165° C. during the addition of the first ten per cent of the terpene and maintained at 165±3° C. throughout the addition of the balance. After all the terpene had been added, the reaction mass was maintained at 165° C. over a period of six hours. It was then cooled to 90° C. and was agitated for 1 hour with 35 pounds of 30% aqueous sodium sulfide solution, the temperature throughout the period of agitation being maintained at approximately 90° C. The agitation was then shut off, a few minutes allowed for separation, and the lower aqueous sulfide layer was run off. The sulfurized terpene was given two additional washes with 35 pounds of 30% aqueous sodium sulfide under the operating conditions outlined above. It was then washed free of sodium sulfide solution with hot brine and finally with hot water. The washed product contained 16.65% sulfur and at 1.0% concentration in oil gave a copper strip test of 1.

The washed product was charged to a still and topped under 60 mm. vacuum to a pot temperature of 170° C. The temperature of 170° C. in the pot at 60 mm. was maintained for a period of 1 hour to insure complete stripping of inert material. It was then filtered hot to containers. The finished product, 105 pounds, contained 33% sulfur, and was a clear reddish-yellow oil having a viscosity of 95 Saybolt second at 210° F. When tested in the copper strip test at 0.5% concentration, a value of 5 was obtained.

## EXAMPLE II

10½ pounds of sulfur were charged to a pot and heated to 145° C. At this temperature, 26 pounds of the terpene hydrocarbons used in Example I above were slowly added over a period of 1 hour at 145° C.±2° C. This temperature was then maintained for an additional 1½ hours. The charge was cooled to 90° C. and was then agitated with 7½ pounds of 30% sodium hydroxide for 1½ hours at a temperature of 90° C. The agitation was then shut off and the caustic layer separated. The product was then agitated with

9 pounds of 24% sodium sulfide solution for 1½ hours at 90° C. After separating the sulfide solution, 24½ pounds of washed product were obtained. This product contained 18.09% sulfur and, when tested at 1% concentration in the copper strip test, did not stain the copper strip, a value of 1.

The clear product was charged to a still and topped to 125° C. under 10 mm. vacuum. 13 pounds of residue, containing 32.9% sulfur, were obtained. This residue was a light reddish-yellow colored oil and has a viscosity of 26 Saybolt seconds at 210° F. At 0.5% concentration, the copper strip test was 3+.

#### EXAMPLE III

9 pounds of sulfur were charged to a pot and heated to 150° C. Then 26 pounds of terpene hydrocarbons of the type used in Example I were added over approximately 1 hour. During the addition of the first 10% of the terpene, the temperature was adjusted to 165° C. and was maintained at 165° C. ± 2° C. during the addition of the last 90% of the terpene. After the addition was complete, the temperature was held at 165° C. for 3 hours. It was then cooled to 90° C., and 6 pounds of 30% aqueous sodium hydroxide were added. The reaction was agitated vigorously with the caustic for 1½ hours at 90° C., then the agitation was shut off and the caustic layer separated. The product was then agitated with 9 pounds of 24% sodium sulfide solution for 1½ hours at 90° C., following which the sulfide solution was separated. 24½ pounds of washed product were obtained. This product contained 16.75% sulfur and, when tested at 1% concentration in the copper strip test, gave a value of 1.

The washed product was charged to a still and topped to 170° C. at 50 mm. 11 pounds of residue were obtained containing 33.96% sulfur. The residue was a light colored reddish-yellow oil having a viscosity of 100.3 Saybolt seconds at 210° F. At 0.5% concentration in the copper strip test, a value of 4 was obtained.

#### EXAMPLE IV

The terpene hydrocarbons, used in this example, consisted of a commercial mixture which contained approximately 40% dipentene, 25% terpinolene, 15% p-cymene, and 20 p-menthane. The latter two ingredients are inert and may be distilled out of the final product.

53 pounds of sulfur were charged to a reactor and heated to a temperature of 150° C. Then 148 pounds of the terpene mixture were added gradually at 145 to 150° C. over 3 hours after which the temperature was maintained at 150° C. for an additional 8 hours. The charge was then cooled to 90° C. and agitated with 46 pounds of 25% sodium sulfide solution for 1 hour at 90° C. The sulfide solution was allowed to settle and was separated. The washing was then twice repeated with equal amounts of sodium sulfide solution. Finally sodium sulfide solution was washed from the product by means of hot brine and hot water. The washed oil, tested at 1.0% concentration, gave a copper strip test of 1. The washed product was charged to a still and topped to a pot temperature of 120° C. under 30 mm. vacuum. It was then filtered into containers. The residue weighed 100 pounds, contained 26% sulfur, and was a light red-yellow colored oil having a viscosity of 47 Saybolt seconds at 210° F. Tested at 0.5% in the copper strip test, it gave a value of 2. This product still contained a slight amount of hydrocarbon material and could be topped further.

#### EXAMPLE V

A second preparation, made in accordance with Example IV, was carried slightly further in the distillation, finishing at 130° C. under 30 mm., and gave a similar product having a sulfur content of 30.65% and a viscosity of 57.4 Saybolt seconds at 210° F. At 0.5% concentration in the copper strip test, a value of 4 was obtained.

10

#### EXAMPLE VI

The terpene hydrocarbons, used in this preparation, consisted of a commercial mixture having the following composition: Dipentene 65%, terpinolene 5%, p-cymene 15%, p-menthane 15%. 15 The last two components are inert and are removed in the topping operation. 9 pounds of sulfur were charged to a reaction pot and heated to 165° C. Then 26 pounds of the terpene mixture were gradually added over 2 hours at 155 to 165° C. After the addition was complete, the temperature was maintained at 160 to 170° C. for an additional 7 hours. The charge was then cooled to 90° C. and washed 3 times with 9 pounds of 24% sodium sulfide solution, agitating each wash for 1 hour at 90° C. The washed product was then charged to a still and topped to 125° C. at 10 mm. vacuum. 14 pounds of residue were obtained. The residue was a somewhat opaque reddish-yellow oil, contained 31.9% sulfur and had a viscosity of 86 Saybolt seconds at 210° F. At 0.5% concentration in the copper strip corrosion test, a value of 4 was obtained.

25

#### EXAMPLE VII

35 To 1988 grams of terpene hydrocarbons of the type used in Example I in an agitated flask, 4 cc. of water and a small amount of sulfur were added, and the temperature was raised to 130° C. The addition of 256 grams of sulfur was started at this temperature. A temperature of 138 to 140° C. was quickly reached and was held there by the addition of 2 cc. more of water which increased the rate of refluxing. As the sulfur was added, some water escaped, and the temperature rose to 45 145° C. where 2 cc. more water were added. It was then possible to complete the addition of the sulfur without any further temperature rise. After the sulfur had all been added, the temperature was raised to 150° C. during one hour and then to 160° C. during 5 hours.

50

The charge was then distilled from a flask immersed in an oil bath in which the temperature was raised to 130° C. Under 10 mm. pressure, 690 grams of distillate were obtained, and the residue in the flask weighed 660 grams. The distillate was largely saturated hydrocarbons which would not react with sulfur. The residue was diluted with an equal volume of a low boiling petroleum hydrocarbon solvent and was washed with agitation with 350 grams of 25% sodium sulfide solution at 95 to 100° C. The sodium sulfide layer was separated and the washing repeated. The solvent was then distilled off on a boiling water bath, and a residue of 550 grams obtained, 60 which had a sulfur content of 24.54% and which did not stain a copper strip under the conditions of the copper strip test.

70

#### EXAMPLE VIII

A repeat preparation was made in exactly the same manner as Example VII insofar as the sulfurization was concerned. The crude sulfurized reaction mass was washed twice with 350 grams of 25% sodium sulfide solution, agitating each wash for 1 hour at 90° C. After separating the

75

second sodium sulfide wash, the charge was distilled under 20 mm. vacuum to a pot temperature of 100° C. 573 grams of distillate and 698 grams of residue were obtained. After filtration, the residue contained 23.98% sulfur and gave a satisfactory copper strip test.

It will be understood that the above examples are given for illustrative purposes solely and many variations can be made therein without departing from the spirit or scope of my invention. For example, other commercial mixtures of terpene hydrocarbons of the character hereinbefore defined may be treated by the same methods. Also, equivalent materials have been prepared from pure dipentene, pure terpinolene and the pure isomeric terpene hydrocarbon of boiling point 187° C. to 188° C. separated from the mixture employed in Example I.

All of the products of the examples, including the products washed with sodium sulfide but not topped, are viscous oils and are yellow or reddish-yellow in color. They are further characterized by the fact that their solutions in petroleum lubricating oils will not attack copper to any appreciable extent or blacken it when subjected to the copper strip test hereinbefore described at 100° C., but will react with and blacken copper in the temperature range of from about 120° C. to about 200° C. The sulfur in the products apparently begins to become active to deposit a black copper sulfide film on a copper strip at temperatures of about 120° C. to about 130° C. In some preparations, this temperature of reactivity may be as low as 110° C., but will always be above 100° C. Most of the sulfur becomes active to blacken copper at temperatures of from about 150° C. to about 170° C., whereas, by 200° C. nearly all of the available sulfur will have reacted. This reactivity of the sulfur at these temperatures appears to be essential for the products to exert their beneficial effect on lubricating oils and particularly to produce extreme pressure properties.

The sulfurized terpene hydrocarbon products of my invention are very effective antioxidants for highly refined mineral oils and for pure oxidizable hydrocarbons in the temperature range of

tion of corrosive oxidation products therein and to a film which is formed on the metals and protects them from corrosion. The sulfurized terpene products of my invention also have excellent extreme-pressure lubricant properties and when blended with chlorinated hydrocarbons make effective and economical bases for hypoid gear lubricants.

The effectiveness of my compounds as oxidation inhibitors at high temperatures may be illustrated by their effect on inhibiting the oxidation of cetane as shown in Table 3. The products employed in these tests were the final topped products.

TABLE 3

## Oxidation of cetane

[Conditions: 1,000 cc. of air per minute through a 33.3 gram sample of cetane in a glass system.]

| Additive       | Conc. Wt. per cent | Temp. | Induction       |
|----------------|--------------------|-------|-----------------|
|                |                    |       | Period, Minutes |
| None.....      |                    | °C.   |                 |
| Example 5..... | 0.075              | 150   | 49              |
| Example 5..... | 0.15               | 150   | over 420        |
| None.....      |                    | 175   | 2               |
| Example 1..... | 0.15               | 175   | 340             |

The value of these non-corrosive sulfurized terpene hydrocarbons as additives for use in extreme-pressure lubricants has been established by the tests outlined in U. S. Army Specification No. 2-105, dated September 10, 1943, and entitled "Lubricant; Gear, Universal (Hypoid and Other Types)".

Table 4 lists the data obtained with the topped products of Example I and Example VIII and also lists comparable results with dibenzyl disulfide which has been accepted as satisfactory by the army for this type service. In all cases the E. P. L. bases tested contain three parts of chlorinated product to one part of the sulfur additive. Two chlorinated products are used: (1) a chlorinated naphthalene and (2) a chlorinated paraffin containing 40% chlorine. The base oil used is a commercial hypoid gear petroleum base oil.

TABLE 4

| Tests <sup>1</sup>                | Base Oil No | 90% Base Oil+7½% Chlorinated naphthalene+2½% of Sulfur Compound |             |             | 90% Base Oil+7½% Chlorinated Paraffin+2½% of Sulfur Compound |             |         |
|-----------------------------------|-------------|-----------------------------------------------------------------|-------------|-------------|--------------------------------------------------------------|-------------|---------|
|                                   |             | Ex. 1                                                           | Ex. 8       | DBDS        | Ex. 1                                                        | Ex. 8       | DBDS    |
| Copper strip at 212° F.....       | Neg.....    | Neg.....                                                        | Neg.....    | Neg.....    | Neg.....                                                     | Neg.....    | Neg.    |
| Copper strip at 300° F.....       | Neg.....    | Pos.....                                                        | Pos.....    | Pos.....    | Pos.....                                                     | Pos.....    | Pos.    |
| SAE Load Carrying Capacity:       |             |                                                                 |             |             |                                                              |             |         |
| 1000 R. P. M. before heating..... |             | 340.....                                                        | 290.....    | 275.....    | 425.....                                                     | 320.....    | 310.    |
| 500 R. P. M. after heating.....   |             | 435.....                                                        | 400.....    | 480.....    | 475.....                                                     | 440.....    | 450.    |
| Emulsion test.....                | 20.....     | 37.....                                                         | 30.....     | 32.....     | 39.....                                                      | 40.....     | 35.     |
| Channel test.....                 | Passes..... | Passes.....                                                     | Passes..... | Passes..... | Passes.....                                                  | Passes..... | Passes. |
| Viscosity S. U. S. 210° F.....    | 83.8.....   | 73.8.....                                                       | 72.7.....   | Passes..... | 80.9.....                                                    | 79.7.....   | 72.2.   |
| V. I.....                         | 75.6.....   | 60.6.....                                                       | 64.7.....   |             | 62.4.....                                                    |             |         |

DBDS—Dibenzyl-Disulfide.

Ex. 1—Sulf. terpene hydrocarbon of Ex. 1 33% S.

Ex. 8—Sulf. terpene hydrocarbon of Ex. 8 24% S.

Chlorinated paraffin—(40% chlorine).

<sup>1</sup> Tests from U. S. Army Spec. No. 2-105.

from about 120° C. to about 200° C., but are ineffective for this purpose at temperatures of 100° C. and below. They are also effective corrosion inhibitors for copper, silver and their alloys when such metals are exposed to oxidizable hydrocarbons in the temperature range of from about 120° C. to about 200° C. This anti-corrosion action appears to be due both to the antioxidant effect on the hydrocarbons which prevents the forma-

tion of corrosive oxidation products therein and to a film which is formed on the metals and protects them from corrosion. The sulfurized terpene products of my invention also have excellent extreme-pressure lubricant properties and when blended with chlorinated hydrocarbons make effective and economical bases for hypoid gear lubricants.

The sulfurized terpene products of my invention are also useful for improving the cetane value of Diesel fuels. For such purpose, they will be added to the Diesel fuel oil in the proportion of from about 0.25% to about 5.00%. In this use, they have an advantage over prior sulfurized terpene products, in that they are non-corrosive to the metals of the fuel system. Their effectiveness for this purpose is illustrated by the

following test data appearing in Table 5 wherein the topped product of Example I was employed:

TABLE 5

| Additive   | Conc. per cent. | Cetane No. | Increase In Cetane No. |
|------------|-----------------|------------|------------------------|
| None       |                 | 47.5       |                        |
| Example I. | .25             | 50.6       | 3.1                    |
| Example I. | .50             | 51.9       | 4.4                    |
| Example I. | 1.00            | 52.5       | 5.0                    |
| Example I. | 2.00            | 55.2       | 7.7                    |

P. O. Powers, in Patent 1,926,648, discloses the preparation of non-corrosive sulfurized terpenes suitable for use as cutting fluids. In order to show more clearly the advantageous properties of the products of my invention over the products of Powers, sulfurized terpenes were made in accordance with the disclosure of Powers and subjected to the copper strip test. First, sulfurized pine oil and sulfurized a-pinene were prepared as follows:

#### Sulfurized pine oil

400 grams of sulfur and 800 grams of pine oil were placed in a flask and heated to a temperature of 178-180° C. At this point a vigorous reaction occurred, and the temperature rose to 190° C. The heat was shut off until the reaction moderated, which took about 5 minutes, and then the heat was again applied and the temperature raised to 210° C. over a period of 30 minutes. The total time was about 1½ hours.

#### Sulfurized a-pinene

400 grams of sulfur and 800 grams of a-pinene were charged to a flask and heated under reflux to 158-160° C. Reflux was maintained at this temperature for about two hours. It took about one hour for the sulfur to dissolve, and the second hour completed the reaction.

Each of these products was then washed by agitating with a 20% aqueous sodium hydroxide solution at 90° C. to 95° C., employing sufficient solution to provide 6 parts of sodium hydroxide for each 100 parts of the sulfurized terpene. Samples of the sulfurized terpene were withdrawn, after washing for 15 minutes, 30 minutes, 60 minutes and 120 minutes, the sodium hydroxide washed therefrom with water and the samples then subjected to the copper strip test hereinbefore described. The results of such tests are shown in Table 6.

TABLE 6

3 hour, 210° F. copper strip test samples at 1.0% and 5.0% conc. in SAE 10 oil

| Wash | Time of Agitation, Min. | Sulfurized Pine Oil Example of Powers |            | Sulfurized a-Pinene Powers Equivalent |      |
|------|-------------------------|---------------------------------------|------------|---------------------------------------|------|
|      |                         | 1.0% Conc.                            | 5.0% Conc. | 1.0%                                  | 5.0% |
| NaOH | 15                      | 10                                    | 10         | 10                                    | 10   |
| Do   | 30                      | 10                                    | 10         | 10                                    | 10   |
| Do   | 60                      | 10                                    | 10         | 10                                    | 10   |
| Do   | 120                     | 10                                    | 10         | 10                                    | 10   |

From these tests, it will be apparent that, while the products of Powers are suitable for cutting oil lubricants, they did not have the required properties in the copper strip test to make them suitable for use in automotive lubricants in the same manner as the compounds of my invention.

In preparing lubricants from my sulfurized

terpene products, the amount of product added to the petroleum oil will generally be in the range of from about 0.05% to about 5%, the particular amount depending upon the use to which the lubricant is to be put and the properties desired therein.

It will thus be apparent that, by my invention, I have provided novel sulfurized terpene products which are suitable for use as antioxidants for hydrocarbon materials in the higher temperature ranges and which are particularly suitable for use in automotive lubricants. It is also apparent that, by my invention, I have provided sulfurized terpene products which are useful in extreme-pressure lubricants where non-corrosive properties are required, and have also provided compounds which are effective for inhibiting bearing corrosion. I believe that I am the first to provide sulfurized terpene products of such character and which are suitable for use in automotive lubricants and the like.

I claim:

1. A sulfurized terpene product obtained by the sulfurization of at least one member of the group consisting of dipentene and terpinolene, followed by washing the sulfurization product at about 85° C. to about 100° C. with an aqueous solution of an alkali metal sulfide of a concentration of about 20% to 30% until a product is obtained which in dilute petroleum oil solution will not form black films on metallic copper at 100° C. but which will form black films on metallic copper at temperatures between 120° C. and 200° C.

2. A sulfurized terpene product obtained by the sulfurization of at least one member of the group consisting of dipentene and terpinolene, washing the sulfurization product at about 85° C. to about 100° C. with an aqueous solution of an alkali metal sulfide of a concentration of about 20% to about 30% until a product is obtained which in 1% concentration in petroleum oil will be substantially non-staining to metallic copper at 100° C., then topping the washed product under vacuum to a pot temperature of from about 100° C. to about 15° C. above the sulfurizing temperature to obtain a product which contains from about 24% to about 36% of chemically combined sulfur and is substantially free of hydrocarbons and which product in dilute petroleum oil solution will not form black films on metallic copper at 100° C. but which will form black films on metallic copper at temperatures between 120° C. and 200° C.

3. A sulfurized terpene product obtained by the sulfurization of a mixture of terpenes the major proportion of which consists of dipentene and terpinolene, followed by washing the sulfurization product at about 85° C. to about 100° C. with an aqueous solution of an alkali metal sulfide of a concentration of about 20% to about 30% until a product is obtained which in dilute petroleum oil solution will not form black films on metallic copper at 100° C. but which will form black films on metallic copper at temperatures between 120° C. and 200° C.

4. A sulfurized terpene product obtained by the sulfurization of a mixture of terpenes the major proportion of which consists of dipentene and terpinolene, washing the sulfurization product at about 85° C. to about 100° C. with an aqueous solution of an alkali metal sulfide of a concentration of about 20% to about 30% until a product is obtained which in 1% concentration in petroleum oil will be substantially non-staining to metallic copper at 100° C., then topping the washed product under vacuum to a pot temperature of from about

100° C. to about 5° C. above the sulfurizing temperature to obtain a product which contains from about 24% to about 36% of chemically combined sulfur and is substantially free of hydrocarbons and which product in dilute petroleum oil solution will not form black films on metallic copper at 100° C. but which will form black films on metallic copper at temperatures between 120° C. and 200° C.

5. The process which comprises heating at least one terpene of the group consisting of dipentene and terpinolene, with sulfur at from about 135° C. to about 180° C. until a substantial proportion of the terpene is sulfurized and washing the reaction mixture at about 85° C. to about 100° C. with an aqueous solution of an alkali metal sulfide of a concentration of about 20% to about 30% until a product is obtained which in 1% concentration in petroleum oil will be substantially non-staining to metallic copper at 100° C.

6. The process which comprises heating at least one terpene of the group consisting of dipentene and terpinolene, with sulfur at from about 135° C. to about 180° C. until a substantial proportion of the terpene is sulfurized and washing the reaction mixture at about 85° C. to about 100° C. with an aqueous solution of sodium sulfide of a concentration of about 20% to about 30% until a product is obtained which in 1% concentration in petroleum oil will be substantially non-staining to metallic copper at 100° C.

7. The process which comprises heating at least one terpene of the group consisting of dipentene and terpinolene, with sulfur at from about 135° C. to about 180° C. until a substantial proportion of the terpene is sulfurized, washing the reaction mixture at about 85° C. to about 100° C. with an aqueous solution of sodium sulfide of a concentration of about 20% to about 30% until a product is obtained which in 1% concentration in petroleum oil will be substantially non-staining to metallic copper at 100° C., then topping the washed product under vacuum to a pot temperature of from about 100° C. to about 5° C. above the sulfurizing temperature until the concentration of sulfur in the product is increased to from about 24% to about 36%.

8. The process which comprises heating a mixture of terpenes the major proportion of which consists of dipentene and terpinolene, with sulfur at from about 135° C. to about 180° C. until a substantial proportion of the terpene is sulfurized and washing the reaction mixture at about 85° C. to about 100° C. with an aqueous solution of an alkali metal sulfide of a concentration of about 20% to about 30% until a product is obtained which in 1% concentration in petroleum oil will be substantially non-staining to metallic copper at 100° C.

9. The process which comprises heating a mixture of terpenes the major proportion of which consists of dipentene and terpinolene, with sulfur at from about 135° C. to about 180° C. until a substantial proportion of the terpene is sulfurized and washing the reaction mixture at about 85° C. to about 100° C. with an aqueous solution of sodium sulfide of a concentration of about 20% to about 30% until a product is obtained which in 1% concentration in petroleum oil will be substantially non-staining to metallic copper at 100° C.

10. The process which comprises heating a mixture of terpenes the major proportion of which consists of dipentene and terpinolene, with sulfur at from about 135° C. to about 180° C. until

a substantial proportion of the terpene is sulfurized, washing the reaction mixture at about 85° C. to about 100° C. with an aqueous solution of sodium sulfide of a concentration of about 20% to about 30% until a product is obtained which in 1% concentration in petroleum oil will be substantially non-staining to metallic copper at 100° C., then topping the washed product under vacuum to a pot temperature of from about 100° C. to about 5° C. above the sulfurizing temperature until the concentration of sulfur in the product is increased to from about 24% to about 36%.

11. The process which comprises heating a mixture of terpenes the major proportion of which consists of dipentene and terpinolene, with from about 1.5 to about 2.1 atoms of sulfur for each mole of the unsaturated terpenes at temperatures of from about 160° C. to about 170° C. until a substantial proportion of the terpenes is sulfurized, washing the reaction mixture at about 85° C. to about 100° C. with an aqueous solution of sodium sulfide containing about 20% to about 30% sodium sulfide until a product is obtained which in 1% concentration in petroleum oil will be substantially non-staining to metallic copper at 100° C., then distilling off hydrocarbons from the washed product under vacuum of about 50 mm. to about 60 mm. to a pot temperature of about 170° C. until the concentration of sulfur in the product is increased to from about 33% to about 34%.

12. The process which comprises heating a mixture of terpenes the major proportion of which consists of dipentene and terpinolene, with from about 1.5 to about 2.1 atoms of sulfur for each mole of the unsaturated terpenes at temperatures of from about 140° C. to about 150° C. until a substantial proportion of the terpenes is sulfurized, washing the reaction mixture at about 85° C. to about 100° C. with an aqueous solution of sodium sulfide containing about 20% to about 30% sodium sulfide until a product is obtained which in 1% concentration in petroleum oil will be substantially non-staining to metallic copper at 100° C., then distilling off hydrocarbons from the washed product under vacuum of about 10 mm. to 30 mm. to a pot temperature of about 120° C. to about 130° C. until the concentration of sulfur in the product is increased to from about 30% to about 34%.

LEE CONE HOLT.

#### REFERENCES CITED

The following references are of record in the file of this patent:

#### UNITED STATES PATENTS

| Number    | Name        | Date           |
|-----------|-------------|----------------|
| 1,926,648 | Powers      | Sept. 12, 1933 |
| 1,926,687 | Palmer      | Sept. 12, 1933 |
| 1,929,955 | Nelson      | Oct. 10, 1933  |
| 1,963,084 | Gardner     | June 19, 1934  |
| 2,012,446 | Edwards     | Aug. 27, 1935  |
| 2,034,665 | Ott         | Mar. 17, 1936  |
| 2,043,961 | Kaufman     | June 9, 1936   |
| 2,045,788 | Maverick    | June 30, 1936  |
| 2,076,875 | Borglin     | Apr. 13, 1937  |
| 2,137,410 | Moran       | Nov. 22, 1938  |
| 2,156,919 | Merriam     | May 2, 1939    |
| 2,246,282 | Zimmer      | June 17, 1941  |
| 2,329,486 | Rummelsburg | Sept. 14, 1943 |
| 2,332,165 | Ott         | Oct. 19, 1943  |

**Certificate of Correction**

Patent No. 2,443,823.

June 22, 1948.

**LEE CONE HOLT**

It is hereby certified that errors appear in the printed specification of the above numbered patent requiring correction as follows: Column 7, line 12, for the word "has" read *had*; line 27, for "was" first occurrence, read *mass*; line 49, for "20 p-menthane" read *20% p-menthane*; column 12, line 29, claim 1, for "20% to 30%" read *20% to about 30%*; and that the said Letters Patent should be read with these corrections therein that the same may conform to the record of the case in the Patent Office.

Signed and sealed this 24th day of August, A. D. 1948.

[SEAL]

**THOMAS F. MURPHY,**  
*Assistant Commissioner of Patents.*